

March 15, 1949.

R. L. HOPKINS

2,464,578

THERMAL TREATMENT OF SHEETS OF MAGNESIC METAL

Filed March 19, 1948



## UNITED STATES PATENT OFFICE

2,464,578

THERMAL TREATMENT OF SHEETS OF  
MAGNESIC METAL

Robert L. Hopkins, Arnold, Pa., assignor to Aluminum Company of America, Pittsburgh, Pa., a corporation of Pennsylvania

Application March 19, 1948, Serial No. 15,818

3 Claims. (Cl. 148—13)

1

This invention relates to improvements in the thermal treatment of rolled sheets of magnesic metal, i. e., magnesium and magnesium base alloy. Its purpose and object is to minimize or prevent distortion of such sheets occurring during thermal treatment. The invention is directed to those thermal treatments in which the individual rolled sheets, or portions cut therefrom, are formed into a stack having two more or less parallel surfaces formed by the outer rolled surfaces of the top and bottom elements of the stack, the other stack surfaces being defined by the edges of the stacked sheet elements. When such stacks are subjected to thermal treatment, they are usually positioned on the outer surface of the bottom element of the stack, and therefore the invention is described herein with reference to a stack so positioned. However, the stack may rest, during thermal treatment, on a stack surface defined by edges of the stacked elements or may be suspended, by a sling or similar means, in the heating chamber. The principles of this invention are useful regardless of the position of the stack during treatment.

For purposes of illustration only reference will be made herein to the accompanying drawing in which—

Fig. 1 is a representation of a stack of sheet elements;

Fig. 2 is a view, partially in section, of one manner in which the methods of this invention may be performed; and

Fig. 3 is a partially sectioned view of one heat flow retarding element useful in the practice of the invention.

As used herein and in the appended claims, the term "magnesic metal" includes magnesium and alloys containing a preponderant amount of such metal, usually 70 per cent by weight or more. There are several types of thermal treatment which may be applied to rolled sheet of magnesic metal. Usually such treatments involve heating the sheets to elevated temperatures, such as 200° to 850° F., and thereafter cooling said sheets. The purpose of the treatment is not involved in this invention, the invention being useful whenever such treatments are performed. When rolled sheets of magnesic metal are so heated and cooled, the sheet is often distorted to such a degree as to destroy the essential flatness of the sheet. In such cases it is often found necessary to resort to further operations, such as stretching, to eliminate the distortion and restore the sheet to its original flatness.

2

It is the purpose of this invention to minimize or prevent such distortion and that end is accomplished by so controlling the flow of heat during thermal treatment as to insure that the greatest rate of heat flow into, or out of, the stack of sheet elements is in a direction substantially normal to the rolled surfaces of said sheet elements. In other words, the flow of heat into, and out of, those stack surfaces which are defined by the edges of the stacked sheet is so retarded that the heat flow is at its greatest rate through those surfaces of the stack which are defined by the rolled surfaces of the top and bottom sheet elements thereof.

15 The principle of the invention will be apparent from a consideration of the sheet stack shown in Fig. 1. Stack surfaces such as A are defined by the edges of the stacked sheet elements. Stack surfaces B are defined by the rolled surfaces of the top and bottom elements of the stack. In thermally treating such a stack in accordance with the principles of this invention the heat flow is retarded at stack surfaces such as A so that the heat flows at its greatest rate in the direction indicated by the arrows. The condition illustrated in Fig. 1 is the cooling cycle of a thermal treatment. During the heating cycle of the treatment the heads of the flow arrows would point in the opposite direction. 20 This control of heating and cooling results in a more uniform temperature in any given sheet than has been obtained heretofore.

35 The arrangement shown in Fig. 2 is typical of a preferred industrial application of the invention. The stack 10 of rolled magnesic metal sheets is supported upon a transporting device consisting of a frame built of structural elements 11 on which is placed a platform 12. All or a portion of this platform may, if desired, be in 40 the form of a grating, as indicated at 13. Also arranged on this transporting device are heat flow retarding elements 14 which in this case are shown in the form of ingots or billets from which magnesic sheet is rolled. Since such ingots are always available in a rolling plant, they are conveniently used for this purpose. The assembly shown in Fig. 2 may readily be lifted and placed in a heating inclosure, such as a furnace. When subjected to heat the passage 45 of the heat into the surface A of the stack 10 will be retarded by the shielding effect of the ingots 14. Also when the assembly is removed from the furnace, or the furnace heat is shut off, to promote cooling of the stacked sheets, the 50 heat stored in the ingots 14 will prevent rapid 55 heat loss in the stack 10.

flow of heat through the stack surfaces A. The result is therefore that the ingots 14 act as barriers and the heat flows most rapidly as indicated in Fig. 1. In the preferred form of the invention, as shown in Fig. 2 hereof, a magnesium plate 18 is inserted between stack 10 and the grating 13 to minimize any marking of the bottom elements of the stack by the grating and also to minimize any distortion effects due to the unequal expansion rates of the grating and the stack.

It will be at once apparent that many various means may be used in the practice of this invention to produce the desired heat flow conditions. For instance, the heat retarding barrier may be formed of material either of substantial volume, such as the ingots 14, or of relatively high insulating properties. A form of device useful for this purpose is the refractory block 15 shown in Fig. 3. Imbedded in block 15 are heating elements 16 to which electrical energy may be supplied through leads 17. Several of such blocks may be used to enclose the stack surfaces A during heating and then, during cooling, energy supplied to the heating elements 16 will insure that flow of heat in a direction normal to stack surfaces A will be retarded. Any other barrier or heat flow retarding device may be used, in effecting, in accordance with this invention, a retarding of the flow of heat into, and out of, those surfaces of the stack which are defined by the edges of the stacked magnesic metal sheets.

The principles of this invention have been successfully used, in the embodiment shown in Fig. 2, to substantially minimize, and often prevent, 35 distortion of rolled magnesic sheet during ther-

mal treatments applied to the stacked sheet and have greatly reduced the need and frequency of later operations designed to restore flatness to the sheet.

- 5 Having thus described my invention, I claim:
1. The method of minimizing distortion of rolled magnesic metal sheet during thermal treatment applied to a stack of such sheets which comprises retarding the flow of heat through 10 those surfaces of said stack which are defined by the edges of said sheets thereby causing a greater rate of heat flow in a direction normal to the other surfaces of said stack.
  2. In a method of thermally treating rolled 15 magnesic metal sheet in which a plurality of said sheets are formed into a stack and submitted to a heating and a cooling cycle, the improvement consisting in placing heat flow retarding elements adjacent those surfaces of said stack 20 which are defined by the edges of the stacked sheet thereby to retard the flow of heat into and from said stack surfaces to a rate less than the rate of heat flow in a direction substantially normal to the stack surfaces defined by the outer 25 rolled surfaces of the top and the bottom elements of said stack.
  3. The step of minimizing distortion of the elements of a stack of rolled magnesic metal sheets during a thermal treatment of said stack, 30 which consists in retarding the flow of heat through the edges of said stacked elements during said treatment.

ROBERT L. HOPKINS.

No references cited.